



US006703344B2

(12) **United States Patent**  
Ueki et al.

(10) **Patent No.:** US 6,703,344 B2  
(45) **Date of Patent:** Mar. 9, 2004

(54) **THERMAL RECORDING MATERIAL**

(75) Inventors: **Shiki Ueki**, Shizuoka-ken (JP);  
**Kazumori Minami**, Shizuoka-ken (JP)

(73) Assignee: **Fuji Photo Film Co., Ltd.**, Kanagawa (JP)

(\*) Notice: Subject to any disclaimer, the term of this patent is extended or adjusted under 35 U.S.C. 154(b) by 102 days.

(21) Appl. No.: **10/173,566**

(22) Filed: **Jun. 18, 2002**

(65) **Prior Publication Data**

US 2003/0013608 A1 Jan. 16, 2003

(30) **Foreign Application Priority Data**

Jun. 18, 2001 (JP) ..... 2001-183893

(51) **Int. Cl.<sup>7</sup>** ..... **B41M 5/30**

(52) **U.S. Cl.** ..... **503/215; 503/226**

(58) **Field of Search** ..... 503/215, 226

(56) **References Cited**

U.S. PATENT DOCUMENTS

5,492,789 A \* 2/1996 Igarashi et al. ..... 430/138

FOREIGN PATENT DOCUMENTS

JP 2000-289337 10/2000

\* cited by examiner

*Primary Examiner*—B. Hamilton Hess

(74) *Attorney, Agent, or Firm*—Sughrue Mion, PLLC

(57) **ABSTRACT**

The invention provides a thermal recording material comprising a support and at least one thermal recording layer disposed on the support, wherein the layer comprises at least one electron-accepting compound, and microcapsules, which encapsulate an electron-donating dye precursor and are formed using a compound represented by the following general formula (I) and a compound represented by the following general formula Formula (II):

Formula (I)



Formula (II)



wherein each of R<sup>1</sup> and R<sup>2</sup> represents an alkyl group; n is an integer selected from 0 to 3; and M represents Na, Mg, K or Ca.

**19 Claims, No Drawings**

## THERMAL RECORDING MATERIAL

## BACKGROUND OF THE INVENTION

## 1. Field of the Invention

The present invention relates to a thermal recording material, more precisely to a thermal recording material having good lightfastness and in particular to a thermal recording material having the advantages of good lightfastness and image fixation.

## 2. Description of the Related Art

Relatively inexpensive and capable of being processed in simple and reliable recording appliances not requiring maintenance, thermal recording materials for forming an image upon being provided with a heat by a thermal head, and the like are widely used in the art. Heretofore, there has been a high demand for high-performance thermal recording materials, for example, with improved high image quality or storage stability and the like. Thus, research relating to color density, image quality, storability, and the like has been performed.

Various types of thermal recording materials have been heretofore known, including, for example, those in which electron-donating leuco-dyes and electron-accepting compounds in which they are reacted to form colors, and those in which diazo compounds such as diazonium salts and couplers in which they are reacted to form colors.

The recent development in the art toward full-color thermal recording materials is noticeable. In general, full-color thermal recording materials have a laminate structure of yellow, magenta and cyan-coloring layers, in which the respective layers are thermally colored to form full-color images.

One example of such full-color thermal recording materials has a laminate structure of color-forming layers (thermal recording layers) comprising an electron-donating leuco-dye and an electron-accepting compound and color-forming layers comprising a diazo compound and a coupler, in which yellow, magenta and cyan color-forming layers are laminated in that order from its top.

One method of improving the storability and the image stability against light and heat of thermal recording materials is to encapsulate the electron-donating leuco-dyes and the diazo compounds in microcapsules. According to this method, the electron-donating leuco-dyes and the diazo compounds in thermal recording materials are isolated from water and bases that may promote their decomposition, and, as a result, the shelf life of the thermal recording materials is prolonged (Tomomasa Usami, et al., "The Journal of the Electrophotography Society of Japan", Vol. 26, No. 2, 1987, pp. 115-125).

In heat-responsive microcapsules, a type of microcapsules in which the glass transition point of the capsule wall is slightly higher than room temperature, the capsule wall is substance-impervious at room temperature but is substance-pervious at a temperature not lower than its glass transition point. Accordingly, when electron-donating leuco-dyes or diazo compounds are encapsulated with this capsule wall and electron-accepting compounds, couplers or bases are outside the microcapsules in the thermal recording material, then the encapsulated electron-donating leuco-dyes or diazo compounds can be kept stable for a long time and a color image can be readily formed by heating the material. In addition, the color image thus formed on the material can be readily fixed thereon through exposure to light (photofixation).

One general method of encapsulating a core substance of electron-donating dye precursors or diazo compounds into microcapsules comprises dissolving the core substance in a hydrophobic solvent (oily phase), followed by emulsifying and dispersing this mixture in an aqueous solution having a water-soluble polymer dissolved therein (aqueous phase) using a homogenizer or the like, with a monomer or a prepolymer, which will be the microcapsule wall, being added to one or both of the oily phase and the aqueous phase, to thereby polymerize the monomer or the prepolymer in the interface between the oily phase and the aqueous phase or precipitate the polymer to form a wall of the polymer compound. The method is described in detail, for example, in "Microcapsules" (by Tomoji Kondo, Nikkan Kogyo Shinbun Publishing, 1970); and "Microcapsules" (by Tamotsu Kondo, et al., Sankyo Publishing, 1977).

However, the above method of microcapsule formation is problematic in that the aqueous solution used forms a lot of bubbles. The bubbles often enter exhaust dusts and therefore lower the production efficiency, and also lower the properties such as the stability of the photographic materials that contain the microcapsules formed according to the method. Therefore, a surfactant that serves as a defoaming agent is generally added to the system of forming microcapsules according to the method. One typical example of the surfactant is sodium dodecylbenzenesulfonate. However, this is still unsatisfactory for completely preventing the generation of bubbles in forming microcapsules when the conditions of this method.

The sensitivity to heat of the microcapsules mentioned above is one important factor thereof. Therefore, if the sensitivity to heat of the microcapsules in one layer of a thermal photographic material is not stable, the quality of the photographic material decreases.

Moreover, when a full color thermal recording material, which is formed by stacking multiple thermal recording layers, uses highly sensitive microcapsules, a problem in that the thermal recording layers comprising microcapsules may generate colors by heat, which is added to cause a color forming reaction in the upper layers. This can cause a mixing of colors and an inferior thermal differentiation. Thus, when thermal recording layers are superimposed, it is preferable to use microcapsules having low heat sensitivity in the lower layers by the support.

For controlling the sensitivity of microcapsules, the reaction temperature in forming the microcapsules is particularly important. In addition, for satisfactorily preventing the generation of bubbles in microcapsule formation, the surfactant alone is unsatisfactory. Therefore, the reaction condition including the reaction temperature in microcapsule formation must be suitably controlled. However, it is difficult to stably form microcapsules of low sensitivity under the reaction conditions which prevent bubbles from being formed, and it has heretofore been difficult to produce full-color thermal recording materials of good thermal differentiation.

## SUMMARY OF THE INVENTION

The present invention is to solve the problems in the prior art noted above, and its object is to provide a thermal recording material having the advantages of superior production suitability, production stability and thermal differentiation.

The means of the invention for solving the problems as above are mentioned below.

Specifically, the invention provides a thermal recording material comprising a support and at least one thermal

recording layer disposed on the support, wherein the layer comprises at least one electron-accepting compound, and microcapsules, which encapsulate an electron-donating dye precursor and are formed using a compound represented by the following general formula (I) and a compound represented by the following general formula (II):



wherein each of R<sup>1</sup> and R<sup>2</sup> represents an alkyl group; n is an integer selected from 0 to 3; and M represents Na, Mg, K or Ca.

The invention also provides a thermal recording material comprising a support and at least one thermal recording layer disposed on the support, wherein the layer comprises at least microcapsules, which encapsulate a diazo compound, and a coupler, for reacting with the diazo compound to produce a color, which microcapsules are formed using a compound represented by the following general formula (I) and a compound represented by the following general formula (II):



wherein each of R<sup>1</sup> and R<sup>2</sup> represents an alkyl group; n is an integer selected from 0 to 3; and M represents Na, Mg, K or Ca.

Moreover, the present invention provides the thermal recording material comprising a support and at least one thermal recording layer disposed on the support, the layer including at least an electron-accepting compound, microcapsules, which encapsulate an electron-donating dye precursor, microcapsules, which encapsulate a diazo compound, and a coupler, for reacting with the diazo compound to produce a color.

In the thermal recording material of the invention, the color density of the microcapsules at a recording energy of 100 mJ/mm<sup>2</sup> is at most 0.20.

#### DETAILED DESCRIPTION OF THE INVENTION

The thermal recording material of the invention is described in detail hereinunder.

##### Thermal Recording Material:

A thermal recording material of the present invention comprises a support and at least one thermal recording layer disposed on the support, the layer including at least an

electron-accepting compound, and microcapsules, which encapsulate an electron-donating dye precursor, and are formed using a compound represented by the following general formula (I) (hereinafter, this may be referred to as a “surfactant (I)”) and a compound represented by the following general formula (II) (hereinafter, this may be referred to as a “surfactant (II)”).

In another aspect, the thermal recording material of the invention comprises, on a support, at least microcapsules, which encapsulate a diazo compound, and a coupler, for reacting with the diazo compound to produce a color, which microcapsules are formed using a compound represented by the following general formula (I) and a compound represented by the following general formula (II):



wherein R<sup>1</sup> represents an alkyl group, and n is from 0 to 3.



wherein each of R<sup>1</sup> and R<sup>2</sup> represents an alkyl group; n is an integer selected from 0 to 3; and M represents Na, Mg, K or Ca.

When forming the microcapsules that encapsulate the electron-donating dye precursor or the diazo compound (both of these will be referred to hereinafter as a “color-forming component”) to be in the thermal recording material of the invention, the surfactants (I) and (II) can be used together to satisfactorily prevent a generation of bubbles in the microcapsule formation. Accordingly, the thermal recording material of the invention has excellent production suitability and performance, such as stability.

To stably form microcapsules of low sensitivity, some amount of heating is necessary. In the invention, it is possible to prevent bubbles from being formed in the microcapsule formation even at high temperatures since the surfactants (I) and (II) are used together therein, and thus microcapsules of low sensitivity can be stably formed.

The thermal recording material of the invention includes at least a thermal recording layer on a support, and the thermal recording layer may have a single-layered or multi-layered structure. If desired, the material may have other layers, such as light-transmittance controlling layer and a protective layer in accordance with necessity.

##### Thermal-Recording Layer:

The thermal recording layer in the invention includes microcapsules, which encapsulate a color-forming component and are formed using the surfactants (I) and (II).

##### Surfactants:

The surfactant (I) is a compound of the following general formula (I):



Formula (I)

5

-continued



(II)-2

wherein R¹ represents an alkyl group. The alkyl group preferably has from 4 to 12 carbon atoms, and more preferably from 6 to 10 carbon atoms.

Specifically, examples of the alkyl group include t-octyl groups, n-octyl groups, n-hexyl groups, t-hexyl groups and n-dodecyl groups. Of those, t-octyl groups and n-octyl groups are preferable, and n-octyl groups are more preferable.

In formula (I), n is an integer selected from 0 to 3. In general, the surfactant (I) for use in the invention is a mixture of compounds of formula (I) where n is an integer selected from 0 to 3, however, the range of n is not specifically defined.

An example of the surfactant (I) is mentioned below. However, the present invention is not limited to this example.



(I)-1

30

The surfactant (II) for use in the invention is a compound of the following general formula (II):



Formula (II)

wherein R² represents an alkyl group. The alkyl group preferably has from 8 to 16 carbon atoms, more preferably from 10 to 14 carbon atoms. The alkyl group may be substituted.

Specifically, examples of the alkyl group include n-octyl groups, t-octyl groups and n-dodecyl groups. Of those, n-dodecyl groups and t-dodecyl groups are preferable, and n-dodecyl groups are more preferable.

In formula (II), M represents Na, Ca, Mg or K, and is preferably Na.

Examples of the surfactant (II) are mentioned below. However, the invention is not limited to these examples.



(II)-1

60

Examples of the high-boiling-point organic solvents are tricresyl phosphate, trioctyl phosphate, octyldiphenyl phosphate, tricyclohexyl phosphate, dibutyl phthalate,

#### Method of Microcapsule Formation:

In the invention, at least an electron-donating dye precursor or a diazo compound is encapsulated in microcapsules.

For encapsulating the color-forming component in microcapsules, any known method may be used. For example, one preferable method of microcapsule formation is interfacial polymerization, which is performed as follows: An electron-donating dye precursor (or diazonium salt compound), which is a color-forming component, is dissolved or dispersed in a slightly water-soluble or water-insoluble organic solvent to prepare an oily phase, this is mixed with an aqueous phase having a water-soluble polymer dissolved therein, and the surfactants (I) and (II) are added to the resulting mixture, which is then emulsified and dispersed by a homogenizer or the like, and heated to cause interfacial polymerizing reaction, which forms a microcapsule wall of the polymer substance at the surface of oil drops. According to this method, microcapsules having a uniform size can be formed within a short period of time, and the recording material containing them has good storability.

In the method of microcapsule formation, the reaction temperature is preferably from 20 to 70°C. and, more preferably from 40 to 70°C. To stably form microcapsules of low sensitivity, the reaction temperature is preferably falls from 60 to 70°C. and, more preferably from 65 to 70°C. If the surfactants (I) and (II) are combined, the method has sufficient anti-foamability, even at a high reaction temperature of from 65 to 70°C., and microcapsules of low sensitivity can be stably formed. Here, "microcapsules of low sensitivity" indicates microcapsules that require high energy (high temperature) to form a color, or in other words, microcapsules, which do not form a color until they are heated to a sufficiently high temperature.

In the present invention, the surfactants are generally dissolved in water. The molar ratio of the surfactant (I) [x] to the surfactant (II) [y], x/y is preferably from 8/2 to 2/8, more preferably from 6/2 to 2/6, and is even more preferably 2/1. When the molar ratio falls is from 8/2 to 2/8, the surfactant mixture prevents bubbles from being formed, from accumulating excessively in the reaction tank, and can perform a sufficient defoaming effect.

The surfactants (I) and (II) may be combined with any other known surfactant, as long as this does not interfere with the effect of the present invention. Examples of the known surfactant include sodium methylnaphthalenesulfonates and 2-ethylhexyl sulfosuccinates.

When the surfactants (I) and (II) are combined with any other known surfactant, the surfactants (I) and (II) preferably comprise at least 50% by weight, more preferably at least 80% by weight of the total amount of the surfactants used.

Examples of the organic solvent include low-boiling-point auxiliary solvents such as acetates, methylene chlorides and cyclohexanones, and/or phosphates, phthalates, acrylates, methacrylates, other carboxylates, aliphatic acid amides, alkylated biphenyls, alkylated terphenyls, alkylated naphthalenes, diarylethanes, chloroparaffins, alcohol solvents, phenol solvents, ether solvents, mono-olefin solvents, and epoxy solvents.

Examples of the high-boiling-point organic solvents are tricresyl phosphate, trioctyl phosphate, octyldiphenyl phosphate, tricyclohexyl phosphate, dibutyl phthalate,

diocetylphthalate, diisopropylphthalate, dicyclohexylphthalate, butyl esters of olefinic acids, diethylene glycol benzoate, dioctyl sebacate, dibutyl sebacate, dioctyl adipate, trioctyl trimellitate, acetyltriethyl citrate, octyl maleate, dibutyl maleate, isoamylbiphenyl, chloroparaffins, diisopropyl naphthalene, 1,1'-ditolylethane, monoisopropylbiphenyl, diisopropylbiphenyl, 2,4-di-tert-amylphenol, N,N-dibutyl-2-butoxy-5-tert-octylaniline, 2-ethylhexyl hydroxybenzoate, polyethylene glycol.

Of those, alcohol solvents, phosphate solvents, carboxylate solvents, alkylated biphenyls, alkylated terphenyls, alkylated naphthalenes, and diarylethanes are especially preferable.

In addition, carbonization inhibitors such as hindered phenols and hindered amines may be added to the high-boiling-point solvents. The high-boiling-point solvents preferably have unsaturated fatty acids, for example,  $\alpha$ -methylstyrene dimers. A commercial product of  $\alpha$ -methylstyrene dimers is, for example, MSD100 (trade name, produced by Mitsui Toatsu Chemical Co. Ltd.).

An example of the water-soluble polymer is polyvinyl alcohol, for example, polyvinyl alcohol, silanol-modified polyvinyl alcohol, carboxy-modified polyvinyl alcohol, amino-modified polyvinyl alcohol, itaconic acid-modified polyvinyl alcohol, styrene-maleic anhydride copolymer, butadiene-maleic anhydride copolymer, ethylene-maleic anhydride copolymer, isobutylene-maleic anhydride copolymer, polyacrylamide, polystyrenesulfonic acid, polyvinylpyrrolidone, ethylene-acrylic acid copolymer, and gelatin. Among these, carboxy-modified polyvinyl alcohol is preferable.

The water-soluble polymer may be combined with a hydrophobic polymer emulsion or latex. Examples of the emulsions latexes include styrene-butadiene copolymers, carboxy-modified styrene-butadiene copolymers and acrylonitrile-butadiene copolymers.

Examples of the polymer substance, which forms the microcapsule walls include polyurethane resin, polyurea resin, polyamide resin, polyester resin, polycarbonate resin, aminoaldehyde resin, melamine resin, polystyrene resin, styrene-acrylate copolymer resin, styrene-methacrylate copolymer resin, gelatin, and polyvinyl alcohol. Among these examples, polyurethane-polyurea resins are particularly preferable.

For example, when a polyurethane-polyurea resin is used for the microcapsule wall material, microcapsule walls are produced as follows: a microcapsule wall precursor such as a polyisocyanate is mixed with an oily medium (oily phase), which will be a core substance to be encapsulated. Furthermore, a second substance (e.g., polyols, polyamines) that reacts with the microcapsule wall precursor to form a capsule wall is mixed in an aqueous solution of a water-soluble polymer (aqueous phase). The oily phase is emulsified and dispersed in the aqueous phase and then heated to cause interfacial polymerization to form a microcapsule wall around every oil drop.

Examples of the polyisocyanate compound are given below, however, the invention is not limited to these examples: diisocyanates such as m-phenylene diisocyanate, p-phenylene diisocyanate, 2,6-tolylene diisocyanate, 2,4-tolylene diisocyanate, naphthalene-1,4-diisocyanate, diphenylmethane-4,4'-diisocyanate, 3,3'-diphenylmethane-4,4'-diisocyanate, xylene-1,4-diisocyanate, 4,4'-diphenylpropane diisocyanate, trimethylene diisocyanate, hexamethylene diisocyanate, propylene-1,2-diisocyanate, butylene-1,2-diisocyanate, cyclohexylene-1,2-diisocyanate, cyclohexylene-1,4-diisocyanate; triisocyanates such as 4,4',

4"-triethylmethane triisocyanate, toluene-2,4,6-triisocyanate; tetraisocyanates such as 4,4'-dimethylphenylmethane-2,2',5,5'-tetraisocyanate; and isocyanate prepolymers such as hexamethylene diisocyanate-trimethylolpropane adduct, 2,4-tolylene diisocyanate-trimethylolpropane adduct, xylylene diisocyanate-trimethylolpropane adduct, tolylene diisocyanate-hexanetriol adduct.

In accordance with necessity, two or more of these examples may be used in combination. Among those examples, those having at least three isocyanate groups in the molecule are particularly preferable.

In the method of microcapsule formation, the organic solvent in which the microcapsule wall precursor and the second substance, with which it reacts, as well as other components such as couplers (and electron-accepting compound), organic bases and sensitizers are dissolved have the same meaning as the organic solvent mentioned hereinabove.

The size of the microcapsules is preferably from 0.1 to 2.0  $\mu\text{m}$ , and more preferably from 0.2 to 1.5  $\mu\text{m}$ .

#### Electron-Donating Dye Precursor:

Examples of the electron-donating dye precursor include triarylmethane compounds, diphenylmethane compounds, thiazine compounds, xanthene compounds, and spiropyran compounds. Of those, triarylmethane compounds and xanthene compounds are preferable, as they form color images of high density.

Specifically, examples of the compounds for the dye precursor include 3,3-bis(p-dimethylaminophenyl)-6-dimethylaminophthalide (crystal violet lactone), 3,3-bis(p-dimethylamino)phthalide, 3-(p-dimethylaminophenyl)-3-(1,3-dimethylindol-3-yl)phthalide, 3-(p-dimethylaminophenyl)-3-(2-methylindol-3-yl)phthalide, 3-(o-methyl-p-diethylaminophenyl)-3-(2-methylindol-3-yl)phthalide, 4,4'-bis(dimethylamino)benzhydrol benzyl ether, N-halophenyl leucoauramine, N-2,4,5-trichlorophenyl leucoauramine, rhodamine-B-anilinolactam, rhodamine(p-nitroanilino)lactam, rhodamine-B-(p-chloroanilino)lactam, 2-benzylamino-6-diethylaminofluorane, 2-anilino-6-diethylaminofluorane, 2-anilino-3-methyl-6-diethylaminofluorane, 3-anilino-3-methyl-6-cyclohexyldiethylaminofluorane, 2-anilino-3-methyl-6-isoamylethylaminofluorane, 2-(o-chloroanilino)-6-diethylaminofluorane, 2-octylamino-6-diethylaminofluorane, 2-ethoxyethylamino-3-chloro-3-diethylaminofluorane, 2-anilino-3-chloro-6-diethylaminofluorane, benzoyl leucomethylene blue, p-nitrobenzyl leucomethylene blue, 3-methylspirodinaphthopyran, 3-ethylspirodinaphthopyran, 3,3'-dichlorospirodinaphthopyran, 3-benzylspirodinaphthopyran, 3-propylspirodibenzopyran.

The coating amount of the electron-donating dye precursor is preferably from 0.1 to 1 g/m<sup>2</sup> in the thermal recording layer, for the same reason as that for the diazonium salt compound mentioned above.

#### Electron-Accepting Compound:

Examples of the electron-accepting compound include phenol derivatives, salicylic acid derivatives, and hydroxybenzoates. Among these examples, bisphenols and hydroxybenzoates are particularly preferable. Specifically, they include the following:

2,2-Bis(p-hydroxyphenyl)propane (bisphenol A), 4,4'-(p-phenylenediisopropylidene)diphenol (bisphenol P), 2,2-bis(p-hydroxyphenyl)pentane, 2,2-bis(p-hydroxyphenyl)ethane, 2,2-bis(p-hydroxyphenyl)butane, 2,2-bis(4'hydroxy-

3',5'-dichlorophenyl)propane, 1,1-(p-hydroxyphenyl)cyclohexane, 1,1-(p-hydroxyphenyl)propane, 1,1-(p-hydroxyphenyl)pentane, 1,1-(p-hydroxyphenyl)-2-ethylhexane, 3,5-di( $\alpha$ -methylbenzyl) salicylic acid and polyvalent metal salts thereof, 3,5-di(tert-butyl)salicylic acid and its polyvalent metal salts, 3- $\alpha$ , $\alpha$ -dimethylbenzylsalicylic acid and polyvalent metal salts thereof, butyl p-hydroxybenzoate, benzyl p-hydroxybenzoate, 2-ethylhexyl p-hydroxybenzoate, p-phenylphenol, and p-cumylphenol.

The electron-accepting compound content of the thermal recording layer is preferably from 0.1 to 30 parts by weight relative to 1 part by weight of the electron-donating dye precursor.

Diazo Compound:

The diazo compound to be encapsulated into microcapsules includes, for example, diazonium salt compounds of the following formula (1):



wherein Ar represents an aromatic group, and X<sup>-</sup> represents an acid anion.

The diazonium salt couples with a coupler, which will be described below, to form a color when heated, or decomposes when exposed to light. Depending on the site and the type of the substituent in the Ar moiety therein, the maximum absorption wavelength of the diazonium salt compound can be controlled.

Examples of the diazonium group to form the salts are 4-(p-tolylthio)-2,5-dibutoxybenzenediazonium, 4-(4-chlorophenylthio)-2,5-dibutoxybenzenediazonium, 4-(N,N-dimethylamino)benzenediazonium, 4-(N,N-diethylamino)benzenediazonium, 4-(N,N-dipropylamino)benzenediazonium, 4-(N-methyl-N-benzylamino)benzenediazonium, 4-(N,N-dibenzylamino)benzenediazonium, 4-(N-ethyl-N-hydroxyethylamino)benzenediazonium, 4-(N,N-diethylamino)-3-methoxybenzenediazonium, 4-(N,N-dimethylamino)-2-methoxybenzenediazonium, 4-(N-benzoylamino)-2,5-dieethoxybenzenediazonium, 4-morpholino-2,5-dibutoxybenzenediazonium, 4-anilinobenzenediazonium, 4-[N-(4-methoxybenzoyl)amino]-2,5-diethoxybenzenediazonium, 4-pyrrolidino-3-ethylbenzenediazonium, 4-[N-(1-methyl-2-(4-methoxyphenoxy)ethyl)-N-hexylamino]-2-hexyloxybenzenediazonium, 4-[N-(2-(4-methoxyphenoxy)ethyl)-N-hexylamino]-2-hexyloxybenzenediazonium, 2-(1-ethylpropoxy)-4-[di-(di-n-butylaminocarbonylmethyl)amino]benzenediazonium, 2-benzylsulfonyl-4-[N-methyl-N-(2-octanoyloxyethyl)]-aminobenzenediazonium.

The maximum absorption wavelength  $\lambda_{\text{max}}$  of the diazonium salt compound is preferably no more than 450 nm, and more preferably from 290 to 440 nm. If  $\lambda_{\text{max}}$  of the compound is longer than 450 nm, the storability of the thermal recording material containing the compound will be poor; but if shorter than the range mentioned above, the image fixation and the image storage stability of the recording material will be reduced and the color of the images formed on the material will be inferior, depending on the combination of the compound with a coupler to be combined with it. The coupler will be described hereinunder.

The diazonium salt compound preferably has at least 12 carbon atoms, a solubility in water is at most 1% and in ethyl acetate of at least 5%.

These diazonium salt compounds may be used either singly or in combinations of two or more, depending on the object of the compounds for color control.

Of the diazonium salts compounds mentioned above, those of the following structural formulae (1) to (3) are more preferable in view of their effect to form dyes of better color hue and their effect to ensure better image fixation and image storage stability.

Structural Formula (1)



Structural Formula (2)



Structural Formula (3)



In the structural formula (1), Ar represents a substituted or unsubstituted aryl group.

Examples of the substituents for the aryl group include alkyl groups, alkoxy groups, alkylthio groups, aryl groups, aryloxy groups, arylthio groups, acyl groups, alkoxy carbonyl groups, carbamoyl groups, carbamido groups, sulfonyl groups, sulfamoyl groups, sulfonamido groups, ureido groups, halogen atoms, amino groups, and heterocyclic groups. These substituents may be further substituted.

The aryl group for Ar preferably has from 6 to 30 carbon atoms, for example, groups of phenyl, 2-methylphenyl, 2-chlorophenyl, 2-methoxyphenyl, 2-butoxyphenyl, 2-(2-ethylhexyloxy)phenyl, 2-octyloxyphenyl, 3-(2,4-di-pentylphenoxyethoxy)phenyl, 4-chlorophenyl, 2,5-dichlorophenyl, 2,4,6-trimethylphenyl, 3-chlorophenyl, 3-methylphenyl, 3-methoxyphenyl, 3-butoxyphenyl, 3-cyanophenyl, 3-(2-ethylhexyloxy)phenyl, 3,4-dichlorophenyl, 3,5-dichlorophenyl, 3,4-dimethoxyphenyl, 3-(dibutylaminocarbonylmethoxy)phenyl, 4-cyanophenyl, 4-methylphenyl, 4-methoxyphenyl, 4-butoxyphenyl, 4-(2-ethylhexyloxy)phenyl, 4-benzylphenyl, 4-amino sulfonylphenyl, 4-N,N-dibutylaminosulfonylphenyl, 4-ethoxycarbonylphenyl, 4-(2-ethylhexylcarbonyl)phenyl, 4-fluorophenyl, 3-acetylphenyl, 2-acetylaminophenyl, 4-(4-chlorophenylthio)phenyl, 4-(4-methylphenyl)thio-2,5-butoxyphenyl, and 4-(N-benzyl-N-methylamino)-2-dodecyloxy carbonylphenyl. However, the invention is not limited to these groups.

These groups may be further substituted with any of alkoxy groups, alkylthio group, substituted phenyl groups, cyano groups, substituted amino groups, halogen atoms, and heterocyclic groups.

In the structural formula (1), R<sup>21</sup> and R<sup>22</sup> each independently represent a substituted or unsubstituted alkyl group, or a substituted or unsubstituted aryl group. R<sup>21</sup> and R<sup>22</sup> may be the same or different.

In case where the group for R<sup>21</sup> and R<sup>22</sup> is substituted, examples of the substituent for the group include an alkoxy group, an alkoxy carbonyl group, an alkylsulfonyl group, a substituted amino group, a substituted amido group, an aryl

group, and an aryloxy group. However, the invention is not limited to those examples.

The alkyl group for  $R^{21}$  and  $R^{22}$  preferably has from 1 to 18 carbon atoms, examples include, groups of methyl, trifluoromethyl, ethyl, propyl, isopropyl, butyl, sec-butyl, t-butyl, pentyl, isopentyl, cyclopentyl, hexyl, cyclohexyl, octyl, t-octyl, 2-ethylhexyl, nonyl, octadecyl, benzyl, 4-methoxybenzyl, triphenylmethyl, ethoxycarbonylmethyl, butoxycarbonylmethyl, 2-ethylhexyloxycarbonylmethyl, 2',4'-diisopentylphenyloxyethyl, 2',4'-di-t-butylphenyloxyethyl, dibenzylaminocarbonylmethyl, 2,4-di-t-amylphenyloxypropyl, ethoxycarbonylpropyl, 1-(2',4'-di-t-amylphenyloxy)propyl, acetylaminooethyl, 2-(N,N-dimethylamino)ethyl, 2-(N,N-diethylamino)propyl, methanesulfonylaminopropyl, acetylaminooethyl, 2-(N,N-dimethylamino)ethyl, and 2-(N,N-diethylamino)propyl.

The aryl group for  $R^{21}$  and  $R^{22}$  preferably has from 6 to 30 carbon atoms, examples include, groups of phenyl, 2-methylphenyl, 2-chlorophenyl, 2-methoxyphenyl, 2-butoxyphenyl, 2-(2-ethylhexyloxy)phenyl, 2-octyloxyphenyl, 3-(2,4-di-t-pentylphenoxyethoxy)phenyl, 4-chlorophenyl, 2,5-dichlorophenyl, 2,4,6-trimethylphenyl, 3-chlorophenyl, 3-methylphenyl, 3-methoxyphenyl, 3-butoxyphenyl, 3-cyanophenyl, 3-(2-ethylhexyloxy)phenyl, 3,4-dichlorophenyl, 3,5-dichlorophenyl, 3,4-dimethoxyphenyl, 3-(dibutylaminocarbonylmethoxy)phenyl, 4-cyanophenyl, 4-methylphenyl, 4-methoxyphenyl, 4-butoxyphenyl, 4-(2-ethylhexyloxy)phenyl, 4-benzylphenyl, 4-aminosulfonylphenyl, 4-N,N-dibutylaminosulfonylphenyl, 4-ethoxycarbonylphenyl, 4-(2-ethylhexylcarbonyl)phenyl, 4-fluorophenyl, 3-acetylphenyl, 2-acetylaminophenyl, 4-(4-chlorophenylthio)phenyl, 4-(4-methylphenylthio)-2,5-butoxyphenyl, and 4-(N-benzyl-N-methylamino)-2-dodecyloxycarbonylphenyl. However, the invention is not limited to those examples.

These groups may be further substituted with alkyloxy groups, alkylthio groups, substituted phenyl groups, cyano groups, substituted amino groups, halogen atoms, and heterocyclic groups.

In the structural formula (2), each of  $R^{24}$ ,  $R^{25}$  and  $R^{26}$  each independently represents a substituted or unsubstituted alkyl group, or a substituted or unsubstituted aryl group, and  $R^{24}$ ,  $R^{25}$  and  $R^{26}$  may be the same or different.

Examples of the substituent for the substituted groups include an alkyl group, an alkoxy group, an alkylthio group, an aryl group, an aryloxy group, an arylthio group, an acyl group, an alkoxy carbonyl group, a carbamoyl group, a carbamido group, a sulfonyl group, a sulfamoyl group, a sulfonamido group, an ureido group, a halogen atom, an amino group, and a heterocyclic group.

The alkyl group for  $R^{24}$ ,  $R^{25}$  and  $R^{26}$  preferably has from 1 to 18 carbon atoms, including, for example, the alkyl groups mentioned hereinabove for  $R^{21}$  and  $R^{22}$  in formula (1), and 1-methyl-2-(4-methoxyphenoxy)ethyl, di-n-butylaminocarbonylmethyl and di-n-55 octylaminocarbonylmethyl groups.

The aryl group for  $R^{24}$ ,  $R^{25}$  and  $R^{26}$  has the same meaning as that for  $R^{21}$  and  $R^{22}$  in formula (1). However, the invention is not limited to these groups.

The groups may be further substituted with alkyloxy groups, alkylthio groups, substituted phenyl groups, cyano groups, substituted amino groups, halogen atoms, and heterocyclic groups.

In the structural formula (2),  $Y$  represents a hydrogen atom, or  $OR^{23}$ , and  $R^{23}$  represents a substituted or unsubstituted alkyl group, or a substituted or unsubstituted aryl group.

Examples of the substituent for the substituted groups include an alkyl group, an alkoxy group, an alkylthio group, an aryl group, an aryloxy group, an arylthio group, an acyl group, an alkoxy carbonyl group, a carbamoyl group, a carbamido group, a sulfonyl group, a sulfamoyl group, a sulfonamido group, an ureido group, a halogen atom, an amino group, and a heterocyclic group.

$Y$  is preferably a hydrogen atom or an alkyloxy group  $OR^{23}$  in which  $R^{23}$  is an alkyl group, in view of color control 10 of the compound.

The alkyl group for  $R^{23}$  has the same meaning as that for  $R^{21}$  and  $R^{22}$  in formula (1), however, the invention is not limited to this.

The aryl group for  $R^{23}$  has the same meaning as that for  $R^{21}$  and  $R^{22}$  in formula (1), however, the invention is not limited to this. The aryl group may be substituted with any of alkyloxy groups, alkylthio groups, substituted phenyl groups, cyano groups, substituted amino groups, halogen atoms, and heterocyclic groups.

In the structural formula (3), each of  $R^{27}$  and  $R^{28}$  independently represents a substituted or unsubstituted alkyl group, or a substituted or unsubstituted aryl group, and  $R^{27}$  and  $R^{28}$  may be the same or different.

Examples of the substituent for the substituted groups include an alkyl group, an alkoxy group, an alkylthio group, an aryl group, an aryloxy group, an arylthio group, an acyl group, an alkoxy carbonyl group, a carbamoyl group, a carbamido group, a sulfonyl group, a sulfamoyl group, a sulfonamido group, an ureido group, a halogen atom, an amino group, and a heterocyclic group.

The alkyl group for  $R^{27}$  and  $R^{28}$  has the same meaning as that for  $R^{21}$  and  $R^{22}$  in formula (1). However, the invention is not limited to this.

The aryl group for  $R^{27}$  and  $R^{28}$  has the same meaning as that for  $R^{21}$  and  $R^{22}$  in formula (1). However, the invention is not limited to this. The aryl group may be substituted with any of alkyloxy groups, alkylthio groups, substituted phenyl groups, cyano groups, substituted amino groups, halogen atoms, and heterocyclic groups.

In the structural formulae (1) to (3),  $X^-$  represents an acid anion. Examples of the acid for the anion include polyfluoroalkylcarboxylic acids having from 1 to 9 carbon atoms, polyfluoroalkylsulfonic acids having from 1 to 9 carbon atoms, boron tetrafluoride, tetraphenylboron, hexafluorophosphoric acid, aromatic carboxylic acids, and aromatic sulfonic acids. Of those, preferred are hexafluorophosphoric acids in view of the crystallinity of the compounds.

Examples of the diazonium salt compounds of the structural formulae (1) to (3) are given below. However, the invention is not limited to these formulae.



**13**

-continued

**14**

-continued

(2)-3 5 (3)-7



(2)-4 10 (3)-8



(3)-1 20 (3)-9



(3)-2 30 (3)-10



(4)-1 35 (3)-3



The diazonium salt compounds of the structural formulae (1) to (3) may be used herein either singly or in combinations of two or more. Further, the diazonium salt compounds of the structural formulae (1) to (3) may be combined with any other known diazonium salt compounds, depending on the objects such as color control and the like.

45 The coating amount of the diazonium salt compound is preferably from 0.05 to 2 g/m<sup>2</sup>, and more preferably from 0.1 to 1 g/m<sup>2</sup> in the thermal recording layer. If the content of the compound in the layer is smaller than 0.05 g/m<sup>2</sup>, the layer might not be able to obtain sufficient color density; but if larger than 2 g/m<sup>2</sup>, the coatability of the coating liquid for the layer may become inferior.

50 Coupler:

55 The coupler that couples with the diazonium salt compound mentioned above to form a dye may be any and every one capable of coupling with the diazonium salt compound to form a dye in a basic and/or neutral atmosphere.

All 4-equivalent couplers that are used in silver halide photographic materials are usable in the invention, and may 60 be selected for use herein depending on the object of the invention including the intended color of the images to be formed.

65 For example, active methylene compounds having a methylene group adjacent to the carbonyl group thereof, phenol derivatives and naphthol derivatives are usable for the couplers in the invention.

## 15

Among them, compounds of the following formula (2) and their tautomers are especially preferred for use herein.



wherein each of  $E^1$  and  $E^2$  independently represents an electron-attracting group, and may be the same or different.

The electron-attracting group is a substituent having a positive Hammett's value  $\delta$ . Preferred examples thereof are acyl group including groups of acetyl, propionyl, pivaloyl, chloroacetyl, trichloroacetyl, trifluoroacetyl, 1-methylcyclopropylcarbonyl, 1-ethylcyclopropylcarbonyl, 1-benzylcyclopropylcarbonyl, benzoyl and 4-methoxybenzoyl, thenoyl groups; an alkoxy carbonyl group including groups of methoxycarbonyl, ethoxycarbonyl, 2-methoxyethoxycarbonyl and 4-methoxyphenoxy carbonyl groups; a carbamoyl group including carbamoyl, N,N-dimethylcarbamoyl, N,N-diethylcarbamoyl, N-phenylcarbamoyl, N-[2,4-bis (pentyloxy)phenyl]carbamoyl, N-[2,4-bis(octyloxy)phenyl]carbamoyl and morpholinocarbonyl groups; an alkylsulfonyl or arylsulfonyl group including groups of methanesulfonyl, benzenesulfonyl and toluenesulfonyl groups; a phosphono group such as a diethylphosphono group; a heterocyclic group including benzoxazol-2-yl, benzothiazol-2-yl, 3,4-dihydroquinazolin-4-on-2-yl and 3,4-dihydroquinazolin-4-sulfon-2-yl groups; a nitro group, an imino group, and a cyano group.

$E^1$  and  $E^2$  may be bonded to each other to form a ring. The ring to be formed by  $E^1$  and  $E^2$  is preferably a 5-membered or 6-membered carbon or hetero ring.

Examples of the couplers are resorcinol, phloroglucine, 2,3-dihydroxynaphthalene, 2,3-dihydroxynaphthalene-6-sodium sulfonate, 1-hydroxy-2-naphthoemorpholinopropylamide, 2-hydroxy-3-naphthalenesodium sulfonate, 2-hydroxy-3-naphthalenesulfonanilide, 2-hydroxy-3-naphthalenesulfonmorpholinopropylamide, 2-hydroxy-3-naphthalenesulfon-2-ethylhexyloxypropylamide, 2-hydroxy-3-naphthalenesulfon-2-ethylhexylamide, 5-acetamido-1-naphthol, 1-hydroxy-8-acetamidonaphthalene-3,6-sodium disulfonate, 1-hydroxy-8-acetamidonaphthalene-3,6-disulfodianilide, 1,5-dihydroxynaphthalene, 2-hydroxy-3-naphthoemorpholinopropylamide, 2-hydroxy-3-naphthoecetyl amide, 2-hydroxy-3-naphthoanilide, 5,5-dimethyl-1,3-cyclohexadione, 1,3-cyclopentanedione, 5-(2-n-tetradecyloxyphenyl)-1,3-cyclohexanedione, 5-phenyl-4-methoxycarbonyl-1,3-cyclohexanedione, 5-(2,5-di-n-octyloxyphenyl)-1,3-cyclohexanedione, N,N'-dicyclohexylbarbituric acid, N,N'-di-n-dodecylbarbituric acid, N-n-octyl-N'-n-octadecylbarbituric acid, N-phenyl-N'-(2,5-di-n-octyloxyphenyl)barbituric acid, N,N'-bis(octadecyloxycarbonylmethyl)barbituric acid, 1-phenyl-3-methyl-5-pyrazolone, 1-(2,4,6-trichlorophenyl)-3-anilino-5-pyrazolone, 1-(2,4,6-trichlorophenyl)-3-benzamido-5-pyrazolone, 6-hydroxy-4-methyl-3-cyano-1-(2-ethylhexyl)-2-pyridone, 2,4-bis(benzoylacetamido)toluene, 1,3-bis(pivaloylacetamidomethyl)benzene, benzoylacetanitrile, thenoylacetanitrile, acetacetanilide, benzoylacetanilide, pivaloylacetanilide, 2-chloro-5-(N-n-butylsulfamoyl)-1-pivaloylacetamidobenzene, 1-(2-ethylhexyloxypropyl)-3-cyano-4-methyl-6-hydroxy-1,2-dihydropyridin-2-one, 1-(dodecyloxypropyl)-3-acetyl-4-methyl-6-hydroxy-1,2-dihydropyridin-2-one, and 1-(4-n-octyloxyphenyl)-3-tert-butyl-5-aminopyrazole.

The details of the couplers are described in JP-A Nos. 4-201483, 7-223367, 7-223368, and 7-323660, and in Japanese

## 16

Patent Application Nos. 5-278608, 5-297024, 6-18669, 6-18670, 7-316280, 8-027095, 8-027096, 8-030799, 8-12610, 8-132394, 8-358755, 8-358756, and 9-069990.

Examples of the couplers of formula (2) are mentioned below, however, the invention is not limited to these examples.



**17**

-continued

**18**

-continued

B-7

5  
10

B-8

15  
20

B-9

25  
30

B-10



35

B-11



45

B-12



50

B-13



65

B-14

B-15

B-16

B-17

B-18

B-19

B-20

B-21

**19**

-continued

**20**

-continued

B-22



B-28

5

10

B-23 15



B-24

25



B-25 30



B-30

35

40

B-26

The coupler content of the thermal recording layer in the invention is preferably from 0.1 to 30 parts by weight relative to 1 part by weight of the diazonium salt compound in the layer.

Other Components:

Organic Base

An organic base is preferably added to the photosensitive thermal recording layer in the invention to promote the coupling reaction of the diazonium salt with the coupler in the layer.

The organic base is preferably in the layer along with the diazonium salt and the coupler, and the organic base may be in the layer singly or in combinations of two or more.

Examples of the organic base include nitrogen-containing compounds such as tertiary amines, piperidines, piperazines, amidines, formamidines, pyridines, guanidines and morpholines. In addition, organic bases described in JP-B 52-46806, JP-A Nos. 62-70082, 57-169745, 60-94381, 57-123086, 58-1347901, and 60-49991, JP-B Nos. 2-24916, and 2-28479, JP-A Nos. 60-165288, and 57-185430 are also usable herein.

Among these examples, piperazines such as N,N'-bis(3-phenoxy-2-hydroxypropyl)piperazine, N,N'-bis[3-(p-methylphenoxy)-2-hydroxypropyl]piperazine, N,N'-bis[3-(p-methoxyphenoxy)-2-hydroxypropyl]piperazine, N,N'-bis



21

(3-phenylthio-2-hydroxypropyl)piperazine, N,N'-bis[3-( $\beta$ -naphthoxy)-2-hydroxypropyl]piperazine, N-3-( $\beta$ -naphthoxy)-2-hydroxypropyl-N'-methylpiperazine, 1,4-bis{[3-(N-methylpiperazino)-2-hydroxy]propoxy}-benzene; morpholines such as N-[3-( $\beta$ naphthoxy)-2-hydroxy]propylmorpholine, 1,4-bis(3-morpholino-2-hydroxypropoxy)benzene, 1,3-bis(3-morpholino-2-hydroxypropoxy)benzene; piperidines such as N-(3-phenoxy-2-hydroxypropyl)piperidine, N-dodecylpiperidine; and guanidines such as triphenylguanidine, tricyclohexylguanidine, dicyclohexylphenylguanidine are particularly preferable.

When the organic base is included in the thermal recording layer, an amount thereof is preferably from 0.1 to 30 parts by weight relative to 1 part by weight of the diazonium salt compound therein.

#### Sensitizer

In addition to the organic base mentioned above, a sensitizer may be added to the thermal recording layer to promoting the color formation in the layer.

The sensitizer acts to increase the color density of the color images formed by heat, or to lower the minimum color-forming temperature of the thermal recording layer. Specifically, it lowers the melting point of the coupler, the organic base and the diazonium salt in the layer, or the softening point of the capsule wall of the microcapsules in the layer, thereby enhancing the reactivity of the diazonium salt, the organic base and the coupler.

Specifically, low-melting-point organic compounds having an aromatic group and a polar group to a suitable degree in the molecule are preferable as the sensitizer. Examples include benzyl p-benzyloxybenzoates,  $\alpha$ -naphthyl benzyl ethers,  $\beta$ -naphthyl benzyl ethers, phenyl  $\beta$ -naphthoates, phenyl  $\alpha$ -hydroxy- $\beta$ -naphthoates,  $\beta$ -naphthol (p-chlorobenzyl) ethers, 1,4-butanediol phenyl ethers, 1,4-butanediol p-methylphenyl ethers, 1,4-butanediol p-ethylphenyl ethers, 1,4-butanediol m-methylphenyl ethers, 1-phenoxy-2-(p-tolylxy)ethanes, 1-phenoxy-2-(p-ethylphenoxy)ethanes, 1-phenoxy-2-(p-chlorophenoxy)ethanes, and p-benzylbiphenyls.

#### Binder

The binder to be in the thermal recording layer may be any known water-soluble polymer compound or latex.

Examples of the water-soluble polymer compound include methyl cellulose, carboxymethyl cellulose, hydroxyethyl cellulose, hydroxypropyl cellulose, starch derivatives, casein, arabic gum, gelatin, ethylene-maleic anhydride copolymer, styrene-maleic anhydride copolymer, polyvinyl alcohol, epichlorohydrin-modified polyamide, isobutylene-maleinsalicylic anhydride copolymer, polyacrylic acid, polyacrylamide, and their modified derivatives; and the latex includes, for example, styrene-butadiene rubber latex, methyl acrylate-butadiene rubber latex, and polyvinyl acetate emulsion.

#### Antioxidant

It is also preferable to add known antioxidants such as those mentioned below to the thermal recording layer for improving the fastness to light and heat of the color images formed and for reducing the yellowness by light of the non-printed area (non-image area) of the recording material after image fixation thereon.

Examples of the antioxidants that are usable herein are described in EP-A Nos. 223739, 309401, 309402, 310551, 310552, and 459416, GP-A No. 3435443, JP-A Nos. 54-48535, 62-262047, 63-113536, 63-163351, 2-262654, 2-71262, 3-121449, 5-61166, and 5-119449, and USP Nos. 4,814,262, and 4,980,275.

22

In the present invention, the mode of using the couplers, the organic bases, the sensitizers and other components is not particularly limited. For example, these components may be solid (1) dispersed; (2) emulsified and dispersed; (3) polymer dispersed; (4) latex dispersed, or (5) encapsulated into microcapsules.

#### Constitution of Thermal Recording Material:

Concrete embodiments of the constitution of full-color thermal recording materials of the invention are described below.

The thermal recording material of the invention is a monochromatic thermal recording material having, on a support, one thermal recording layer specifically defined herein, or a full-color thermal recording material having a laminate layer structure of multiple thermal recording layers formed on a support in which at least one thermal recording layer of the present invention. In the full-color thermal recording material, it is desirable that at least one thermal recording layer is a photo-fixing recording layer that contains a diazonium salt compound and a coupler capable of reacting with the diazonium salt compound to form a color.

particularly when the full-color thermal recording material has cyan, yellow and magenta-forming thermal recording layers, it is desirable that the first thermal recording layer nearest to the support contains a leuco-type color former of an electron-donating dye precursor and an electron-accepting compound, and the second and third thermal recording layers contain a diazo-type color former.

For example, the thermal recording material may be formed by embodiments expressed by the following (a)-(c).

(a) A recording material comprising a laminated structure of; a photo-fixing recording layer that contains the low sensitivity microcapsules of the present invention which encapsulate a diazonium salt compound (maximum absorption wavelength of  $365\pm40$  nm) therein, and a coupler capable of reacting with the diazonium salt compound to form a dye (first recording layer A); and a photo-fixing recording layer that contains a diazonium salt compound (maximum absorption wavelength of  $420\pm40$  nm) and a coupler capable of reacting with the diazonium salt compound to form a dye (second recording layer B). This recording material may have a light transmittance-controlling layer and a protective layer on the laminate structure, according to necessity.

(b) A recording material comprising a laminated structure of; a recording layer that contains the low sensitivity microcapsules of the present invention, which encapsulate an electron-donating dye precursor, and an electron-accepting compound (first recording layer A); a photo-fixing recording layer that contains a diazonium salt compound (maximum absorption wavelength of  $365\pm40$  nm), and a coupler capable of reacting with the diazonium salt compound to form a dye (second recording layer B); and a photo-fixing recording layer that contains a diazonium salt compound (maximum absorption wavelength of  $420\pm40$  nm) and a coupler capable of reacting with the diazonium salt compound to form a dye (third recording layer C) laminated on the support in that order. This recording material may have a light transmittance-controlling layer and a protective layer on the laminate structure, according to necessity.

(c) A recording material comprising a laminated structure of; a photo-fixing recording layer that contains the low sensitivity microcapsules of the invention, which encapsulate a diazonium salt compound (maximum absorption wavelength of at most 350 nm), and a

coupler capable of reacting with the diazonium salt compound to form a dye (first recording layer A); a photo-fixing recording layer that contains a diazonium salt compound (maximum absorption wavelength of  $365\pm40$  nm), and a coupler capable of reacting with the diazonium salt compound to form a dye (second recording layer B); and a photo-fixing recording layer that contains a diazonium salt compound (maximum absorption wavelength of  $420\pm40$  nm) and a coupler capable of reacting with the diazonium salt compound to form a dye (third recording layer C) laminated on a support in that order. The recording material may have a light transmittance-controlling layer and a protective layer on the laminate structure, according to necessity.

When a surfactant such as that mentioned hereinabove is used in forming the low sensitivity microcapsules of the present invention to be in the laminate layer structure of the thermal recording material, the microcapsules can be formed stably. Therefore, in the thermal recording material of the present invention, it is preferable that the thermal recording layer with the microcapsules therein be further coated with at least one other thermal recording layer on its recording surface, and it is more preferable that the thermal recording layer with the microcapsules therein is nearest to the support (lowermost layer).

Methods of forming full-color images on the embodiments (b) and (c) are described below.

First, the third recording layer (C) is heated, and the diazonium salt is reacted with the coupler therein to form a dye. Next, the recording material is exposed to light of which the emission center wavelength is  $430\pm30$  nm, whereby the non-reacted diazonium salt compound in the layer C is decomposed and the image, which has been formed is photo-fixed. Then, the recording material is exposed to heat sufficient to form a dye in the second recording layer (B), and the diazonium salt compound in the layer (B) is reacted with the coupler therein to form a dye. In this stage, the layer C is also strongly heated, but the diazonium salt compound therein has been already decomposed (that is, the image formed has been photo-fixed), and has lost its color-forming ability. Next, the recording material is exposed to light of which the emission center wavelength is  $360\pm20$  nm, whereby the diazonium salt compound in the layer B is decomposed and the image formed is photo-fixed. Finally, the recording material is exposed to heat sufficient to form a dye in the first recording layer (A). In this stage, the layers (B) and (C) are also strongly heated, but the diazonium salt compounds therein have been already decomposed and have lost their color-forming ability. In cases where the thermal recording layer of the invention is the layer (A), it is preferable that the sensitivity of the microcapsules therein be no more than  $60\text{ mJ/mm}^2$  in terms of the recording energy to form yellow of O.D.=1.5, and more preferably no more than  $55\text{ mJ/mm}^2$ . In cases where the thermal recording layer of the invention is the layer (B), it is preferable that the sensitivity of the microcapsules therein be no more than  $100\text{ mJ/mm}^2$  in terms of the recording energy to form magenta of O.D.=1.5, and more preferably no more than  $95\text{ mJ/mm}^2$ . Preferably, the sensitivity to heat of the microcapsules with an electron-donating dye precursor or a diazonium salt compound encapsulated therein in the thermal recording material of the invention is low such that the color density of the image formed, in terms of the optical density, O.D. at a recording energy of  $100\text{ mJ/mm}^2$ , is no more than 0.2. More preferably, the sensitivity to heat of the microcapsules with an electron-donating dye precursor or a diazonium salt compound encapsulated

therein in the lowermost layer (A) in the thermal recording material of the invention is low such that the color density of the image (cyan image) formed, in terms of the optical density, O.D. at recording energy of  $100\text{ mJ/mm}^2$ , is no more than 0.2. Controlling the sensitivity to heat of the microcapsules of the invention in the layer (A) (lowermost layer) to the range as above makes it possible to prevent the layer (A) from forming a color when heat is applied to the layer (B). Accordingly, color mixing in the image formed on the recording material of the invention is prevented, and the thermal differentiation in the recording material is improved.

In cases where all the recording layers (A, B and C) in the recording material are diazo-type recording layers, the layers (A) and (B) must be photo-fixed after processed for color image formation, but the layer (C), which is finally processed for color image formation last, does not necessarily require photo-fixing.

The light source for photo-fixation may be selected from any known light sources. Examples include various fluorescent lamps, xenon lamps and mercury lamps. A light source of having an emission spectrum is almost the same as the absorption spectrum of the diazonium salt compound used in the recording material is especially preferable, as it enables high-efficiency photo-fixation.

#### 25 Other Layers:

The thermal recording material of the present invention that has one or more thermal recording layers on a support preferably also has a light transmittance-controlling layer and a protective layer.

#### Light Transmittance-Controlling Layer:

The light transmittance-controlling layer contains a UV absorbent precursor, in which the precursor does not function as a UV absorbent before the layer is exposed to light necessary for image fixation. Therefore, before being exposed to light for image fixation, the light transmittance of the layer is high. When the photo-fixing thermal recording layers are exposed to light for image fixation thereon, the light transmittance-controlling layer transmits the light for image fixation well and transmits visible light well, and therefore does not interfere with image fixation on the recording layers. The UV absorbent precursor in the light transmittance-controlling layer is preferably encapsulated into microcapsules.

Examples of the compounds that may be in the light transmittance-controlling layer are given in JP-A No. 9-1928.

After the thermal recording layers have been exposed to light for image fixation thereon, the UV absorbent precursor in the light transmittance-controlling layer receives light or heat and becomes able to function as a UV absorbent. Accordingly, almost all light falling within a UV range is absorbed by the UV absorbent in the light transmittance-controlling layer, and the UV light transmittance of the layer is lowered. As a result, the lightfastness of the image-recorded material is improved, but since the UV absorbent does not absorb visible light, the visible light transmittance of the image-recorded material does not substantially change.

At least one light transmittance-controlling layer may be 60 in the thermal recording material of the invention, and most preferably, between the thermal recording layer and the outermost protective layer. However, the light transmittance-controlling layer may also serve as a protective layer. The characteristics of the light transmittance-controlling layer may be suitably determined, depending on the characteristics of the thermal recording layers in the recording material.

A coating liquid for forming the light transmittance-controlling layer (coating liquid for light transmittance-controlling layer) may be prepared by mixing the components mentioned above. The coating liquid can be applied onto the recording layer-coated material by any known coating method using, for example, a bar coater, an air knife coater, a blade coater or a curtain coater. The light transmittance-controlling layer may be formed simultaneously with the thermal recording layers; or after the coating liquids for the thermal recording layers have been applied onto a support and been dried thereon, the coating liquid for the light transmittance-controlling layer may be applied onto the recording layers.

A dry weight of the light transmittance-controlling layer formed is preferably from 0.8 to 4.0 g/m<sup>2</sup>.

#### Protective Layer:

The protective layer contains a binder, and also a pigment, a lubricant, a surfactant, a dispersant, a fluorescent brightener, a metal soap, a hardener, a UV absorbent, a crosslinking agent, and the like.

The binder may be any, which has not inhibit the barrier property of the protective layer or the workability of the layer. Examples include polyvinyl alcohol, methyl cellulose, carboxymethyl cellulose, hydroxyethyl cellulose, starches, gelatin, arabic gum, casein, styrene-maleic anhydride copolymer hydrolyzate, ethylene-maleic anhydride copolymer hydrolyzate, isobutylene-maleic anhydride copolymer hydrolyzate, polyvinyl alcohol, modified polyvinyl alcohol, and polyacrylamide.

In addition to the above, synthetic rubber latexes and synthetic resin emulsions are also usable as the binder. For example, styrene-butadiene rubber latex, acrylonitrile-butadiene rubber latex, methyl acrylate-butadiene rubber latex, and polyvinyl acetate emulsion.

The binder content of the protective layer is preferably from 10 to 500% by weight, more preferably from 50 to 400% by weight of the pigment in the layer.

For improving the waterproofness of the protective layer, a crosslinking agent combined with a catalyst for promoting its reaction is effective. Examples of the crosslinking agent include epoxy compounds, blocked isocyanates, vinylsulfone compounds, aldehyde compounds, methylol compounds, boric acids, carboxylic acid anhydrides, silane compounds, chelate compounds and halide compounds, and those capable of controlling the pH of the coating liquid for the protective layer from 6.0 to 7.5 are preferable. The catalyst may be any known acid or metal salt. For it, those capable of controlling the pH of the coating liquid to be from 6.0 to 7.5 are also preferred.

Any known organic or inorganic pigment may be used in the protective layer. Specifically, examples of the pigment include calciumcarbonate, aluminium hydroxide, barium sulfate, titanium oxide, talc, agalmatolite, kaolin, calcined kaolin, amorphous silica, colloidal silica, urea-formalin resin powder, polyethylene resin powder, and benzoguanamine resin powder. One or more of these may be in the layer singly or in combinations of two or more.

Preferable examples of the lubricant that may be in the protective layer are zinc stearate, calcium stearate, paraffin wax, and polyethylene wax.

A surfactant is added to the coating liquid for the protective layer so that the protective layer can be uniformly formed on the thermal recording layers. Preferable examples thereof are alkali metal sulfosuccinates and fluorine-containing surfactants, and specifically, they are sodium salts and ammonium salts of di(2-ethylhexyl)sulfosuccinic acid and di(n-hexyl)sulfosuccinic acid.

The coating liquid for forming the protective layer (coating liquid for protective layer) may be obtained by mixing the above-mentioned components. If desired, a release agent, wax and a water repellent may be added thereto.

To produce the thermal recording material of the invention, the coating liquid may be applied to the thermal recording layers formed on a support to thereby form the protective layer thereon, by any ordinary coating method. For example, a bar coater, an air knife coater, a blade coater or a curtain coater may be used.

The protective layer may be formed simultaneously with the thermal recording layers and the light transmittance-controlling layer. Alternatively, the protective layer may be formed on the recording layers after the coating liquids for the thermal recording layers are applied onto a support and dried.

The dry weight of the protective layer is preferably from 0.2 to 7 g/m<sup>2</sup>, more preferably from 1 to 4 g/m<sup>2</sup>. If the dry weight is lower than 0.2 g/m<sup>2</sup>, the protective layer might not be able to maintain water resistance; but if higher than 7 g/m<sup>2</sup>, the thermal sensitivity of the recording material might be significantly lowered. After the protective layer has been formed, it may be optionally calendered.

#### Interlayer:

When the thermal recording layer comprises multiple layers, providing an interlayer between the neighboring thermal recording layers is preferable. Like the protective layer, the interlayer may contain a binder and also a pigment, a lubricant, a surfactant, a dispersant, a fluorescent brightener, a metal soap, a UV absorbent, and the like. The binder in the interlayer may be the same as that in the protective layer.

#### Support:

The support for the thermal recording layer of the invention is made of, for example, polyethylene terephthalate (PET), polyethylene naphthalate (PEN), triacetyl cellulose (TAC), paper, plastic resin-laminated paper, or synthetic paper. For transparent thermal recording materials, the support must be transparent. The transparent support may be a synthetic polymer film, including, for example, polyester films of polyethylene terephthalate or polybutylene terephthalate, cellulose triacetate film, and polyolefin films of polypropylene or polyethylene.

The support maybe a single-layered support or a laminated support.

The thickness of the synthetic polymer films for the support is preferably from 25 to 300  $\mu$ m, and more preferably from 100 to 250  $\mu$ m.

The synthetic polymer films may be colored in any desired manner. Examples of coloring methods include <1> previously kneading a dye in resin before the resin is formed into films, and the dye-containing resin is formed into a film; or <2> dissolving a dye in a suitable solvent to prepare a dye solution, and applying this onto a transparent colorless resin films in an ordinary coating method, and dried thereon. Examples of the coating and drying methods include gravure coating, roller coating and wire coating. Among these examples, films of polyethylene terephthalate or polyethylene naphthalate containing a blueing dye are preferable. The films may be thermally processed, stretched or processed for static charge prevention.

The thermal recording layers, the protective layer, the light transmittance-controlling layer and the interlayer mentioned above may be formed on a support by any known coating method, and dried thereon. Examples of the known coating method include blade coating, air knife coating,

gravure coating, roll coating, spraying, dipping, and bar coating. If desired, the back surface of the support, which is not coated with the thermal recording layers may be coated with a back coat layer, or an adhesive layer (sealant layer) combined with a release layer.

## EXAMPLES

The invention is described in more detail with reference to the following Examples. However, these examples are not intended to restrict the scope of the present invention.

### Example 1

## Preparation of Aqueous Solution of Phthalated Gelatin

32 parts by weight of phthalated gelatin (trade name: MGP GELATIN, provided by Nippi Collagen), 0.9143 parts by weight of 1,2-benzothiazolin-3-one (3.5% solution in methanol provided by Daito Chemical Industry), and 367.1 parts by weight of ion-exchanged water were mixed and dissolved at 40° C. to prepare an aqueous solution of phthalated gelatin.

## Preparation of Aqueous Solution of Alkali-Processed Gelatin

25.5 parts by weight of alkali-processed low-ion gelatin (trade name: #750 GELATIN, provided by Nitta Gelatin), 0.7286 parts by weight of 1,2-benzothiazolin-3-one (3.5% solution in methanol, provided by Daito Chemical Industry), 0.153 parts by weight of calcium hydroxide, and 143.6 parts by weight of ion-exchanged water were mixed and dissolved at 50° C. to prepare an aqueous solution of alkali-processed gelatin.

## Preparation of Coating Liquid (a) for Yellow Thermal Recording Layer

## Preparation of Diazonium Salt Compound-Containing Microcapsule Dispersion (a)

2.2 parts by weight of a diazonium salt compound (A) mentioned below (maximum absorption wavelength: 420 nm), 2.2 parts by weight of a diazonium salt compound (B) mentioned below (maximum absorption wavelength: 420 nm), 4.8 parts by weight of monoisopropylbiphenyl, 4.8 parts by weight of diphenyl phthalate, and 0.4 parts by weight of diphenyl(2,4,6-trimethylbenzoyl) phosphine oxide (trade name: LUCILIN TPO, provided by BASF Japan), were added to 16.1 parts by weight of ethyl acetate and uniformly dissolved under heat at 40° C.

11.0 parts by weight of a capsule wall-forming material, which is a mixture of xylylene diisocyanate/trimethylolpropane adduct and xylylene diisocyanate/bisphenol A adduct (trade name: TAKENATE D119N (50 wt. % solution in ethyl acetate) provided by Takeda Chemical Industry), was added to this mixture and uniformly stirred to prepare a mixture (I).

16.3 parts by weight of ion-exchanged water and 0.34 parts by weight of an aqueous solution of 50 wt. % alkyl-glucoside surfactant (trade name: SCRAPHAG-8, provided by Nippon Seika) were added to 58.6 parts by weight of the aqueous solution of phthalated gelatin to separately prepare a mixture (II).

The mixture (I) was added to the mixture (II), and emulsified and dispersed at 40° C. by a homogenizer (provided by Nippon Seiki Seisakusho). 20 parts by weight

of water was added to the resulting emulsion and uniformly mixed. Afterwards, this mixture was stirred and ethyl acetate was removed therefrom at 40° C., while performing the encapsulating reaction for three hours. Next, an ion-exchange resin Amberlite (6.2 parts by weight of IRA68 (trade name), provided by Organo, and 12.4 parts by weight of IRC50 (trade name) provided by Organo) was added thereto, and further stirred for 1 hour. Next, the ion-exchange resin was removed through filtration, and the resulting dispersion was processed to have a solid content of 20%, thus obtaining a diazonium salt compound-containing microcapsule dispersion (a). The grain size of the micro-capsules formed was measured with a grain size analyzer (trade name: LA-700, provided by Horiba Seisakusho); the median diameter was found to be 0.36  $\mu\text{m}$ .



### 35 Preparation of Coupler Emulsion (a):

9.9 parts by weight of a coupler (C) mentioned below, 9.9 parts by weight of triphenylguanidine (provided by Hodogaya Chemical), 20.8 parts by weight of 4,4'-(m-phenylenediisopropylidene)diphenol (trade name: BISPHENOL M, provided by Mitsui Petrochemical), 3.3 parts by weight of 3,3,3',3'-tetramethyl-5,5',6,6'-tetra(1-propyloxy)-1,1'-spirobisisindane (provided by Sankyo Chemical), 13.6 parts by weight of 4-(2-ethyl-1-hexyloxy)benzenesulfonamide (provided by Manac), 6.8 parts by weight of 4-n-pentyloxybenzenesulfonamide (provided by Manac), and 4.2 parts by weight of calcium dodecylbenzenesulfonate (trade name: PIONIN A-41-C, 70% solution in methanol, provided by Takemoto Yushi) were dissolved in 33.0 parts by weight of ethyl acetate to prepare a mixture (III).

206.3 parts by weight of the aqueous solution of alkali-processed gelatin was mixed with 107.3 parts by weight of ion-exchanged water to separately prepare a mixture (IV).

55 The mixture (III) was added to the mixture (IV), and  
 emulsified and dispersed at 40° C. by a homogenizer  
 (provided by Nippon Seiki Seisakusho). The resulting coupler  
 emulsion was heated under reduced pressure to remove  
 60 ethyl acetate, and then processed to have a solid content of  
 26.5% by weight. The grain size of the grains in the coupler  
 emulsion was measured with a grain size analyzer (trade  
 name: LA-700, provided by Horiba Seisakusho), and a  
 median diameter thereof was 0.21  $\mu\text{m}$ .

9 parts by weight of 26.5 wt. % SBR latex (trade name: SN-307, 48 wt. % solution, provided by Sumika ABS Latex) was added to 100 parts by weight of the coupler emulsion, and uniformly stirred to prepare a coupler emulsion (a).

29



Preparation of Coating Liquid (a) for Yellow Thermal Recording Layers

The diazonium salt compound-containing microcapsule dispersion (a) and the coupler emulsion (a) were mixed in a coupler/diazonium salt compound ratio by weight of 2.2/1 to prepare a coating liquid (a) for yellow thermal recording layers.

Preparation of Coating liquid (b) for Magenta Thermal Recording Layers

Preparation of Diazonium Salt Compound-Containing Microcapsule Dispersion (b)

2.8 parts by weight of a diazonium salt compound (D) mentioned below (its maximum absorption wavelength is 365 nm) 2.1 parts by weight of diphenyl phthalate, 6.1 parts by weight of phenyl 2-benzoyloxybenzoate, 3.7 parts by weight of TMPT, and 0.1 parts by weight of calcium dodecylbenzenesulfonate (trade name: PIONIN A-41-C, 70% solution in methanol, provided by Takemoto Yushi), were added to 15.1 parts by weight of ethyl acetate and uniformly dissolved under heat.

Capsule wall-forming materials, 2.5 parts by weight of a mixture of xylylene diisocyanate/trimethylolpropane adduct and xylylene diisocyanate/bisphenol A adduct (trade name: TAKENATE D119N (50 wt. % solution in ethyl acetate), provided by Takeda Chemical Industry), and 6.8 parts by weight of xylylene diisocyanate/trimethylolpropane adduct (trade name: TAKENATE D110N (75 wt. % solution in ethyl acetate), provided by Takeda Chemical Industry), were added to the above mixture and uniformly stirred to prepare a mixture (V). p 21.0 parts by weight of ion-exchanged water was added to 55.3 parts by weight of the aqueous solution of phthalated gelatin, and mixed to separately prepare a mixture (VI).

The mixture (V) was added to the mixture (VI), and emulsified and dispersed at 40° C. by a homogenizer (by Nippon Seiki Seisakusho). 30 parts by weight of water was added to the resulting emulsion and uniformly mixed. This was stirred at 40° C. for 3 hours to form microcapsules, while removing ethyl acetate. Next, an ion-exchange resin Amberlite (4.1 parts by weight of IRA68 (trade name), provided by Organo, and 8.2 parts by weight of RC50, (trade name), provided by organo) was added thereto, and stirred for 1 hour. The ion-exchange resin was removed through filtration, and the resulting dispersion was processed to have a solid content of 20%. This is a diazonium salt compound-containing microcapsule dispersion (b). The grain size of the microcapsules formed was measured with a grain size

30

analyzer (trade name: LA-700, provided by Horiba Seisakusho); was found to be 0.43  $\mu$ m the median diameter. Diazonium Salt Compound D:



Preparation of Coupler Emulsion (b)

11.9 parts by weight of a coupler (E) mentioned below, 14.0 parts by weight of triphenylguanidine (provided by Hodogaya Chemical), 14.0 parts by weight of 4,4'-(m-phenylenediisopropylidene)diphenol (trade name: BISPHENOL M, provided by Mitsui Petrochemical), 14 parts by weight of HF-209 (trade name, provided by Honshu Chemical), 3.5 parts by weight of 3,3,3',3'-tetramethyl-5,5',6,6'-tetra(1-propyloxy)-1,1'-spiroindane (provided by San-kyo Chemical), 3.5 parts by weight of 2,2'-(2-methinepropylidene)-bis(4,6-dimethylphenyl), 1.7 parts by weight of tricresyl phosphate, 0.8 parts by weight of diethyl maleate, and 4.5 parts by weight of calcium dodecylbenzenesulfonate (trade name: PIONIN A-41-C, 70% solution in methanol, provided by Takemoto Yushi) were dissolved in 36.9 parts by weight of ethyl acetate to prepare a mixture (VII).

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9

31

## Preparation of Coating Liquid (c) for Cyan Thermal Recording Layers

32

### Electron-Donating Dye Precursor F

### Preparation of Electron-Donating Dye Precursor-Containing Microcapsule Dispersion (c)

5.0 parts by weight of an electron-donating dye precursor (F) mentioned below, 8.0 parts by weight of a mixture of 1-methylpropylphenyl-phenylmethane and 1-(1-methylpropylphenyl)-2-phenylethane (tradename: HISOL 15 SAS-310, provided by Nippon Oil), and 8.0 parts by weight of IRGAPER 2140 (trade name, provided by Ciba Speciality Chemicals) were added to 18.1 parts by weight of ethyl acetate, and uniformly dissolved under heat.

Capsule wall-forming materials, 7.2 parts by weight of xylylene diisocyanate/trimethylolpropane adduct (trade name: TAKENATE D110N (75 wt. % solution in ethyl acetate), provided by Takeda Chemical Industry) and 5.3 parts by weight of polymethylene-polyphenyl polyisocyanate (trade name: MILLIONATE MR-200, provided by Nippon Polyurethane Industry) were added to the mixture, and uniformly stirred to prepare a mixture (IX).

9.5 parts by weight of ion-exchanged water, 0.17 parts by weight of an aqueous solution of 50 wt. % alkylglucoside surfactant (trade name: SCRAPH AG-8, provided by Nippon Seika—which is surfactant (I) in the present invention), and 0.43 parts by weight of an aqueous solution of 10 wt. % sodium dodecylbenzenesulfonate (this is surfactant (II) in the invention) were added to 28.8 parts by weight of the aqueous solution of phthalated gelatin to separately prepare a mixture (X).

The mixture (IX) was added to the mixture (X), and emulsified and dispersed at 40° C. by a homogenizer (provided by Nippon Seiki Seisakusho). 50 parts by weight of water and 0.12 parts by weight of diethylenetriamine were added to the resulting emulsion and uniformly mixed. This was stirred at 65° C. for 3 hours to form microcapsules, while removing ethyl acetate. The resulting microcapsule dispersion was processed to have a solid content of 33 wt. %. The grain size of the microcapsules formed was measured with a grain size analyzer (trade name: LA-700, provided by Horiba Seisakusho), and the median diameter was found to be 1.00  $\mu\text{m}$ .

3.7 parts by weight of an aqueous solution of 25 wt. % sodium dodecylbenzenesulfonate (trade name: NEOPELEX F-25, provided by Kao) and 4,4'-bistriazinylaminostilbene-2,2'-disulfone derivative (trade name: KAYCALL BXNL, provided by Nippon Soda) were added to 100 parts by weight of the microcapsule dispersion, and uniformly stirred. This is an electron-donating dye precursor-containing microcapsule dispersion (c).



### Preparation of Electron-accepting Compound Dispersion (c)

30.1 parts by weight of ion-exchanged water, 15 parts by  
25 weight of 4,4'-(p-phenylenediisopropylidene)diphenol  
(trade name: BISPHENOL P, provided by Mitsui  
Petrochemical), and 3.8 parts by weight of an aqueous  
solution of 2 wt. % sodium 2-ethylhexylsuccinate were  
added to 11.3 parts by weight of the aqueous solution of  
30 phthalated gelatin, and dispersed in a ball mill overnight to  
prepare a dispersion. A solid content thereof was 26.6% by  
weight.

45.2 parts by weight of the alkali-processed aqueous solution was added to 100 parts by weight of the dispersion, 35 and stirred for 30 minutes. Ion-exchanged water was added to this to make the resulting dispersion have a solid content of 23.5% by weight. This is an electron-accepting compound dispersion (c).

## Preparation of Coating Liquid (c) for Cyan Thermal Recoding Layers

The electron-donating dye precursor-containing micro-capsule dispersion (c) and the electron-accepting compound dispersion (c) were mixed in an electron-accepting compound/electron-donating dye precursor of 10/1 ratio by weight to prepare a coating liquid (c) for cyan thermal recording layers.

## Preparation of Coating Liquid for Interlayers

30 100.0 parts by weight of an aqueous solution of alkali-  
processed low-ion gelatin (trade name: #750 GELATIN,  
provided by Nitta Gelatin), 2.857 parts by weight of 1,2-  
benzothiazolin-3-on (3.5 wt. % solution in methanol, by  
55 Daito Chemical Industry), 0.5 parts by weight of calcium  
hydroxide, and 521.643 parts by weight of ion-exchanged  
water were mixed and dissolved at 50° C. to prepare an  
aqueous gelatin solution for interlayers.

10.0 parts by weight of the aqueous gelatin solution for  
60 the interlayer, 0.05 parts by weight of sodium  
(4-nonylphenoxytrioxyethylene)butylsulfonate (provided  
by Sankyo Chemical, aqueous 2.0 wt. % solution), 1.5 parts  
by weight of boric acid (aqueous 4.0 wt. % solution), 0.19  
parts by weight of an aqueous solution of 5 wt. % polysty-  
65 renesulfonic acid (partially neutralized with potassium  
hydroxide), 4.53 parts by weight of H-603M (trade name,  
provided by Wako Pure Chemicals), and 0.67 parts by

33

weight of ion-exchanged water were mixed to prepare a coating liquid for interlayers.

Preparation of Coating Liquid for Light Transmittance-Controlling Layes

Preparation of UV Absorbent Precursor-Containing Microcapsule Dispersion

14.5 parts by weight of a UV absorbent precursor, [2-allyl-6-(2H-benzotriazol-2-yl)-4-t-octylphenyl] benzenesulfonate, 5.0 parts by weight of 2,2'-t-octylhydroquinone, 1.9 parts by weight of tricresyl phosphate, 5.7 parts by weight of  $\alpha$ -methylstyrene dimer (trade name: MSD-100, provided by Mitsui Chemical), and 0.45 parts by weight of calcium dodecylbenzenesulfonate (trade name: PIONIN A-41-C (70% solution in methanol), provided by Takemoto Yushi) were added to 71 parts by weight of ethyl acetate, and uniformly dissolved. 54.7 parts by weight of a capsule wall-forming material, xylylene diisocyanate/trimethylolpropane adduct (trade name: TAK-ENATE D110N (75 wt. % solution in ethyl acetate), provided by Takeda Chemical Industry) was added to To the mixture, and uniformly stirred to prepare a UV absorbent precursor-containing mixture.

8.9 parts by weight of an aqueous 30 wt. % phosphoric acid solution and 532.6 parts by weight of ion-exchanged water were mixed with 52 parts by weight of itaconic acid-modified polyvinyl alcohol (trade name: KL-318, provided by Kuraray) to prepare an aqueous PVA solution for UV absorbent precursor-containing microcapsule dispersion.

The UV absorbent precursor-containing mixture was added to 516.06 parts of the aqueous PVA solution for UV absorbent precursor-containing microcapsule dispersions, and emulsified and dispersed at 20° C. by a homogenizer (by Nippon Seiki Seisakusho). 254.1 parts by weight of ion-exchanged water was added to the resulting emulsion and uniformly mixed. This was stirred at 40° C. for 3 hours to form microcapsules. Next, 94.3 parts by weight of an ion-exchange resin Amberlite (trade name: MB-3, provided by Organo) was added thereto, and stirred for 1 hour. Next, the ion-exchange resin was removed through filtration, and the resulting microcapsule dispersion was processed to have a solid content of 13.5%. The grain size of the microcapsules formed was measured with a grain size analyzer (trade name: LA-700, provided by Horiba Seisakusho), and the median diameter was found to be  $0.23 \pm 0.05 \mu\text{m}$ . 859.1 parts by weight of the microcapsule dispersion was mixed with 2.416 parts by weight of carboxy-modified styrene-butadiene latex (tradename: SN-307 (aqueous 48 wt. % solution), provided by Sumitomo Norgatta) and 39.5 parts by weight of ion-exchanged water to prepare a UV absorbent precursor-containing microcapsule dispersion.

Preparation of Coating Liquid for Light Transmittance-Controlling Layers

1000 parts by weight of the UV absorbent precursor-containing microcapsule dispersion, 5.2 parts by weight of MEGAFAC F-120 (by Dai-Nippon Ink Chemical Industry, aqueous 5 wt. % solution), 7.75 parts by weight of aqueous 4 wt. % sodium hydroxide solution, and 73.39 parts by weight of sodium (4-nonylphenoxytrioxyethylene) butylsulfonate (by Sankyo Chemical, aqueous 2.0 wt. % solution) were mixed to prepare a coating liquid for light transmittance-controlling layers.

Preparation of Coating Liquid for Protective Layer

Preparation of Polyvinyl Alcohol Solution for Protective Layers

160 parts by weight of vinyl alcohol-alkyl vinyl ether copolymer (trade name: EP-130, provided by Denki Kagaku

34

Kogyo), 8.74 parts by weight of a mixture of sodium alkylsulfonate and polyoxyethylene alkyl ether phosphate (trade name: NEOSCORE CM-57 (aqueous 54 wt. % solution) provided by Toho Chemical Industry), and 3832 parts by weight of ion-exchanged water were mixed and dissolved at 90° C. for 1 hour to prepare a uniform polyvinyl alcohol solution for protective layers.

Preparation of Pigment Dispersion for Protective Layers

8 parts by weight of barium sulfate (trade name: BF-21F, having a barium sulfate content of at least 93%, provided by Sakai Chemical Industry) was mixed with 0.2 parts by weight of anionic, special polycarboxylic acid-type polymer surfactant (trade name: POISE 532A (aqueous 40 wt. % solution), provided by Kao) and 11.8 parts by weight of ion-exchanged water, and dispersed by a dino mill. Measured with a grain size analyzer (trade name: LA-910, provided by Horiba Seisakusho), the median diameter of the grain size of the grains in the dispersion was at most 0.15  $\mu\text{m}$ .

8.1 parts by weight of colloidal silica (trade name: SNOWTEX O (aqueous 20 wt. % dispersion), provided by Nissan Chemical) was added to 45.6 parts by weight of the dispersion to prepare a pigment dispersion for protective layers.

Preparation of Matting Agent Dispersion for Protective Layers

220 parts by weight of wheat starch (trade name: WHEAT STARCH S, provided by Shinshin Foods) was mixed with 3.81 parts by weight of an aqueous dispersion of 1,2-benzisothiazolin-3-on (trade name: PROXEL BD, provided by ICI) and 1976.19 parts by weight of ion-exchanged water, and uniformly dispersed to prepare a matting agent dispersion for protective layer.

Preparation of Coating Blend for the Protective Layer

1000 parts by weight of the polyvinyl alcohol solution for protective layer, 40 parts by weight of W-1016 (trade name: MEGAFAC F-120, provided by Dai-Nippon Ink Chemical Industry) (aqueous 5 wt. % solution), 50 parts by weight of sodium (4-nonylphenoxytrioxyethylene)butylsulfonate (by Sankyo Chemical, aqueous 2.0 wt. % solution), 49.87 parts by weight of the pigment dispersion for protective layer, 16.65 parts by weight of the matting agent dispersion for protective layer, and 48.7 parts by weight of zinc stearate dispersion (trade name: HIDRIN 115, aqueous 20.5 wt. % solution, provided by Chukyo Yushi) were uniformly mixed to prepare a coating blend for protective layer.

Formation of Undercoat Layer-Coated Support

Preparation of Coating Liquid for Undercoat Layers

40 parts by weight of enzyme-degraded gelatin (mean molecular weight 10000; PAGI viscosity 1.5 mP·s (15 mP); PAGI jelly strength 20 g) was added to 60 parts by weight of ion-exchanged water, and dissolved while stirring at 40° C. to prepare an aqueous gelatin solution for undercoat layers.

On the other hand, 8 parts by weight of water-swellable synthetic mica (aspect ratio 1000; trade name: SOMASHIF ME100, provided by Corp Chemical) was mixed with 92 parts by weight of water, and wet-milled in a visocomill to

35

prepare a mica dispersion having a volume-average grain size of 2.0  $\mu\text{m}$ . Water was added to the mica dispersion to make it have a mica content of 5% by weight, and uniformly mixed. This is the desired mica dispersion.

Next, 120 parts by weight of water and 556 parts by weight of methanol were added to 100 parts by weight of the aqueous 40 wt. % gelatin solution for undercoat layers at 40° C., and well stirred and mixed. Then, 208 parts by weight of the 5 wt. % mica dispersion was added to this mixture stirred and mixed well, and 9.8 parts by weight of 1.66 wt. % polyethylene oxide-type surfactant was added thereto. With the liquid temperature kept at 35 to 40° C., 7.3 parts by weight of an epoxy compound serving as a gelatin hardener was added to it to prepare a coating liquid (5.7 wt. %) for undercoat layers.

#### Formation of Undercoat Layer-Coated Support

Using a double-disc refiner, wood pulp of LBPS and LBPK, 50/50 parts by weight was beaten to a Canadian freeness of 300 ml. To this were added 0.5 parts by weight, in terms of absolute dry weight relative to the pulp—the same definition applies to the other additives, of epoxidated behenamide, 1.0 part by weight of anionic polyacrylamide, 1.0 part by weight of aluminium sulfate, 0.1 parts by weight of polyamide-polyamine-epichlorohydrin, and 0.5 parts by weight of cationic polyacrylamide. Using a Fourdrinier machine, the paper stock thus-prepared was made into base paper having a unit weight of 114 g/m<sup>2</sup>, and this was calendered to have a thickness of 100  $\mu\text{m}$ .

The base paper were subjected to a corona discharge treatment on both surfaces thereof. Polyethylene resin was extruded through a melt extruder onto the base paper to form a matted resin layer thereon having a thickness of 36  $\mu\text{m}$  (the resin-coated surface of the paper is referred to as a "back") Next, also using a melt extruder, the other surface of the paper, which is opposite to the resin-coated back, was coated with polyethylene resin containing 10% by weight of anatase-type titanium dioxide and a slight amount of ultramarine, to thereby form a glossy resin layer thereon having a thickness of 50  $\mu\text{m}$  (this surface is referred to as "face"). The polyethylene resin-coated back of the paper was subjected to corona discharge treatment, and an aqueous dispersion of an antistatic agent, aluminium oxide (trade name: ALUMINA SOL 100, provided by Nissan Chemical Industry)/silicon dioxide (trade name: SNOWTEX O, provided by Nissan Chemical Industry)=½ (by weight) was applied to the back to form a layer thereon having a dry weight of 0.2 g/m<sup>2</sup>. Next, the polyethylene resin-coated face of the paper was also subjected to corona discharge treatment, and the coating liquid for undercoat layer was applied to the face to form a undercoat layer thereon. The coating amount of the undercoat layer was 0.26 g/m<sup>2</sup> in terms of mica therein. Thus, a undercoat layer-coated support was formed

#### Support Coating with Coating Liquids for Thermal Recording Layers

The undercoat layer-coated face of the support was coated continuously with the coating liquid (c) for cyan thermal recording layer, the coating liquid for interlayers (interlayer A), the coating liquid (b) for magenta thermal recording layers, the coating liquid for interlayers (interlayer B), the coating liquid (a) for yellow thermal recording layers, the coating liquid for light transmittance-controlling layers, and the coating liquid for protective layers, to form the seven layers on the face of the support in that order, and then

36

continuously dried at 30° C. and 30% RH and at 40° C. and 30% RH to form a full-color thermal recording material.

The coating amount of the coating liquid (a) for yellow thermal recording layers was 0.078 g/m<sup>2</sup> in terms of the solid content of the diazonium salt compound (A) in the liquid; that of the coating liquid (b) for magenta thermal recording layers was 0.206 g/m<sup>2</sup> in terms of the solid content of the diazonium salt compound (D) therein; and that of the coating liquid (c) for cyan thermal recording layers was 0.355 g/m<sup>2</sup> in terms of the solid content of the electron-donating dye precursor (F) therein.

The coating amount of the coating liquid for interlayers A was 3.34 g/m<sup>2</sup> in terms of the solid content of the layer; that for interlayer B was 2.39 g/m<sup>2</sup> in terms of the solid content thereof; the coating amount of the coating liquid for light transmittance-controlling layer was 2.35 g/m<sup>2</sup> in terms of the solid content of the layer; and that of the coating liquid for protective layer was 1.39 g/m<sup>2</sup> in terms of the solid content thereof.

#### Formation of Back Coat Layer

##### Preparation of Coating Liquid for Back Coat Layer A (Uppermost Layer)

###### Preparation of Aqueous Solution of Alkali-Processed Gelatin for Back Coat Layers

25 parts by weight of alkali-processed gelatin (trade name: PBLC GELATIN, provided by PB Gelatins, England), 75 parts by weight of alkali-processed gelatin (trade name: PR GELATIN, provided by Miyagi Chemical Industry), 2.95 parts by weight of 1,2-benzothiazolin-3-on (3.5 wt. % solution in methanol, by Daito Chemical Industry), and 450 parts by weight of ion-exchanged water were mixed and dissolved at 50° C. to prepare an aqueous, alkali-processed gelatin solution for back coat layers.

###### Preparation of Silica Dispersion

100 parts by weight of amorphous silica (trade name: 40 MIZUKASIL P526A, provided by Mizusawa Chemical Industry) was mixed with 2.5 parts by weight of aqueous 40% sodium hexametaphosphate, 10 parts by weight of a polycarboxylic acid-type dispersant (trade name: POISE 520A, provided by Kao) and 880 parts by weight of ion-exchanged water and stirred to prepare a silica dispersion having a mean grain size of 6  $\mu$  (measured with LA700 (trade name), provided by Horiba Seisakusho).

###### Preparation of Coating Liquids

50 1000 parts by weight of the aqueous, alkali-processed gelatin solution for back coat layers, 4500 parts by weight of the silica dispersion, 25 parts by weight of an aqueous solution of 70% sulfosuccinate-type surfactant (trade name: RAPISOL B90, provided by Nippon Yushi), and 1000 parts by weight of ion-exchanged water were mixed to prepare a coating liquid for back coat layer A.

##### Preparation of Coating Liquid for Back Coat Layer B (Under Layer)

60 1000 parts by weight of the aqueous, alkali-processed gelatin solution for back coat layer, 2 parts by weight of an aqueous solution of 70% sulfosuccinate-type surfactant (trade name: RAPISOL B90, provided by Nippon Yushi), 300 parts by weight of ion-exchanged water, and 200 parts by weight of AQUABRID EM-13 (by Daicel Chemical Industry) were mixed to prepare a coating liquid for back coat layers B.

## Formation of Back Coat Layers

The surface of the support opposite to that coated with the thermal recording layers of the full-color thermal recording material was coated continuously with back coat layer B and back coat layer A in that order, and dried at 30° C. and 30% RH and at 40° C. and 30% RH, like the thermal recording layers as above, to thereby form the two-layered back coat layer.

The coating amounts of the back coat layer B and the back coat layer A were 10 g/m<sup>2</sup> and 1.0 g/m<sup>2</sup>, respectively, in terms of the solid content of the layer.

## Formation of Release Sheet

## Coating Release Sheet Substrate with Release Layer

A biaxially-stretched foam film produced by stretching pigment-containing polyethylene terephthalate (trade name: CRYSPER, provided by Toyobo, which is a foam PET film flattened with rolls to have a thickness of 100 µm or 75 µm) was used as a release sheet substrate. Using a Mayer bar, this sheet was coated with a silicone release agent (trade name: LTC-750A, provided by Toray Dow Corning Silicone) to form thereon a release layer having a dry weight of 0.2±0.05 g/m<sup>2</sup>, thus obtaining a release sheet used herein.

## Back Printing on Release Sheet

Codes for the registration marks for prints in TA printers, the print formats, the customers, and the like, were printed on the surface of the release sheet opposite to that coated with the release layer. The printing ink was prepared by mixing 100 parts by weight of PANACIA CVL-SP805 (trade name, provided by Dai-Nippon Ink Chemical), 8 parts by weight of PANACIA CVL HARDERNER #10 (trade name, provided by Dai-Nippon Ink Chemical) and 10 parts by weight of USL FILM REINFORCE (trade name, provided by Dai-Nippon Ink Chemical) followed by diluting the resulting blend with a diluent, DIREJUCER UR #2 (trade name, provided by Dai-Nippon Ink Chemical). Using the blend ink, the codes were printed on that surface of the release sheet in a mode of gravure printing.

## Lamination

2 parts by weight of a crosslinking agent, polyfunctional aromatic isocyanate (trade name: CORONATE L, provided by Nippon Polyurethane Industry) was added to 100 parts by weight of an acrylic adhesive (trade name: BPS-4849-40N, provided by Toyo Ink), and well stirred. Using an applicator, this was applied onto the release agent-coated surface of the release sheet to form thereon an adhesive layer having a dry weight of 15±2 g/m<sup>2</sup>. The adhesive-coated release sheet was laminated on the back coat layer of the full-color thermal recording material, which has the release sheet on its back, thus obtaining the thermal recording material of Example 1.

## Comparative Example 1

A full-color thermal recording material of Comparative Example 1 was produced in the same manner as in Example 1, except that “0.17 parts by weight of the aqueous 50 wt. % alkylglucoside surfactant (trade name: SCRAPH AG-8, provided by Nippon Seika, which is surfactant (I)) and 0.43 parts by weight of the aqueous 10 wt. % solution of sodium dodecylbenzenesulfonate (this is surfactant (II))” were changed to “1.28 parts by weight of an aqueous 10 wt. % sodium dodecylbenzenesulfonate solution” in preparing the electron-donating dye precursor-containing microcapsule dispersion (c) of Example 1.

## Comparative Example 2

A full-color thermal recording material of Comparative Example 2 was produced in the same manner as in Comparative Example 1, except that the reaction temperature in preparing the electron-donating dye precursor-containing microcapsule dispersion (c) of Comparative Example 1 was changed from “65° C.” to “55° C.”.

## Evaluation

## Thermal Recording

Images were recorded on the full-color thermal recording materials obtained above, according to the condition mentioned below.

A printer, TRT-21 (trade name, provided by Nagano Nippon Musen) was used to record a yellow image on the recording materials, in which the printing power and the pulse width were controlled so that the recording energy could be from 0 to 71 mJ/mm<sup>2</sup> per the unit area.

Next, the materials were exposed to a UV lamp (emission center wavelength 420 nm, power 40 W) for 10 seconds to fix the yellow image on the yellow thermal recording layer. Then, the printing power and the pulse width were controlled so that the recording energy from the thermal head could vary according to the printing steps as in Table 1 below and a magenta color was recorded.

Finally, the materials were exposed to a UV lamp (emission center wavelength 365 nm, power 40 W) for 15 seconds to fix the magenta image on the magenta thermal recording layer; then the printing power and the pulse width were so controlled that the recording energy from the thermal head could be from 0 to 137 mJ/mm<sup>2</sup> and a cyan image was recorded.

## Measurement of Color Density

In every printing step of Table 1, the cyan color density of the image-recorded materials was measured with a Macbeth densitometer (trade name, provided RD-918 by Macbeth). The results are given in Table 1.

TABLE 1

| Printing Step | Recording Energy mJ/mm <sup>2</sup> | Comparative |           |           |
|---------------|-------------------------------------|-------------|-----------|-----------|
|               |                                     | Example 1   | Example 1 | Example 2 |
| 0             | 0.0                                 | 0.11        | 0.11      | 0.11      |
| 1             | 26.5                                | 0.11        | 0.11      | 0.11      |
| 2             | 37.6                                | 0.11        | 0.11      | 0.11      |
| 3             | 48.8                                | 0.11        | 0.11      | 0.11      |
| 4             | 59.9                                | 0.11        | 0.11      | 0.11      |
| 5             | 71.0                                | 0.11        | 0.11      | 0.11      |
| 6             | 82.1                                | 0.10        | 0.11      | 0.11      |
| 7             | 93.2                                | 0.11        | 0.11      | 0.25      |
| 8             | 104.3                               | 0.24        | 0.23      | 0.55      |
| 9             | 115.5                               | 0.62        | 0.60      | 0.98      |
| 10            | 126.6                               | 1.05        | 1.08      | 1.47      |
| 11            | 137.7                               | 1.53        | 1.53      | 1.74      |
| 12            | 148.8                               | 1.76        | 1.74      | 1.86      |
| 13            | 159.9                               | 1.84        | 1.82      | 1.85      |
| 14            | 171.1                               | 1.84        | 1.82      | 1.85      |

As in Table 1, the full-color thermal recording material of Example 1 had a low cyan density, and the thermal differentiation in yellow, magenta and cyan therein was good.

The full-color thermal recording material of Comparative Example 1 also had a low cyan density like that of Example 1. However, the electron-donating dye precursor-containing microcapsule dispersion (c) was difficult to stably prepare, since the reaction system foamed a lot when forming the microcapsules and a lot of bubbles stayed in the upper part of the reactor, and the productivity of the recording material of Comparative Example 1 was low.

Furthermore, in Comparative Example 2, foaming could be suppressed during the encapsulating reaction for the electron-donating dye precursor-containing microcapsule dispersion (c). However, the cyan density of the image-recorded material was high, and the thermal differentiability of the recording material of Comparative Example 2 is not good.

The invention provides a thermal recording material having the advantages of excellent production applicability, production stability and thermal differentiation.

What is claimed is:

1. A thermal recording material comprising a support and at least one thermal recording layer disposed on the support, wherein the layer comprises at least one electron-accepting compound, and microcapsules, which encapsulate an electron-donating dye precursor and are formed using a compound represented by the following general formula (I) and a compound represented by the following general formula (II):



wherein each of R<sup>1</sup> and R<sup>2</sup> represents an alkyl group; n is an integer selected from 0 to 3; and M represents Na, Mg, K or Ca.

2. The thermal recording material according to claim 1, further comprising at least one thermal recording layer disposed on the support, the layer including at least microcapsules, which encapsulate a diazo compound, and a coupler, for reacting with the diazo compound to produce a color.

3. The thermal recording material according to claim 2, wherein a color density of the microcapsules at a recording energy of 100 mJ/mm<sup>2</sup> is no more than 0.20.

4. The thermal recording material according to claim 2, wherein the molar ratio of the surfactant (I) represented by the formula (I) [x] to the surfactant (II) represented by the formula (II) [y], x/y, is from 8/2 to 2/8.

5. The thermal recording material according to claim 1, wherein a color density of the microcapsules at a recording energy of 100 mJ/mm<sup>2</sup> is no more than 0.20.

6. The thermal recording material according to claim 1, wherein R<sup>1</sup> in formula (I) is an alkyl group having from 4 to 12 carbon atoms.

7. The thermal recording material according to claim 1, wherein R<sup>1</sup> in formula (I) is one of a t-octyl group and a n-octyl group.

8. The thermal recording material according to claim 1, wherein R<sup>2</sup> in formula (II) is an alkyl group having from 8 to 16 carbon atoms.

9. The thermal recording material according to claim 1, wherein R<sup>2</sup> in formula (II) is one of an n-dodecyl group and a t-dodecyl group.

10. The thermal recording material according to claim 1, wherein the reaction temperature for forming the microcapsules is from 60 to 70° C.

5 11. The thermal recording material according to claim 1, wherein the molar ratio of the surfactant (I) represented by the formula (I) [x] to the surfactant (II) represented by the formula (II) [y], x/y, is from 8/2 to 2/8.

12. A thermal recording material comprising a support and at least one thermal recording layer disposed on the support, wherein the layer comprises at least microcapsules, which encapsulate a diazo compound, and a coupler, for reacting with the diazo compound to produce a color, which microcapsules are formed using a compound represented by the following general formula (I) and a compound represented by the following general formula (II):



wherein each of R<sup>1</sup> and R<sup>2</sup> represents an alkyl group; n is an integer selected from 0 to 3; and M represents Na, Mg, K or Ca.

13. The thermal recording material according to claim 12, wherein a color density of the microcapsules at a recording energy of 100 mJ/mm<sup>2</sup> is no more than 0.20.

40 14. The thermal recording material according to claim 12, wherein R<sup>1</sup> in formula (I) is an alkyl group having from 4 to 12 carbon atoms.

15. The thermal recording material according to claim 12, wherein R<sup>1</sup> in formula (I) is one of a t-octyl group and a n-octyl group.

45 16. The thermal recording material according to claim 12, wherein R<sup>2</sup> in formula (II) is an alkyl group having from 8 to 16 carbon atoms.

17. The thermal recording material according to claim 12, wherein R<sup>2</sup> in formula (II) is one of an n-dodecyl group and a t-dodecyl group.

50 18. The thermal recording material according to claim 12, wherein the reaction temperature for forming the microcapsules is from 60 to 70° C.

60 19. The thermal recording material according to claim 12, wherein the molar ratio of the surfactant (I) represented by the formula (I) [x] to the surfactant (II) represented by the formula (II) [y], x/y, is from 8/2 to 2/8.